

May 22, 1934.

F. P. GARDNER

1,959,757

METHOD OF CLEANING FIBERS

Filed Sept. 20, 1930

2 Sheets-Sheet 1



INVENTOR  
Frederick P. Gardner  
BY  
Darby & Darby  
ATTORNEYS

May 22, 1934.

F. P. GARDNER

1,959,757

METHOD OF CLEANING FIBERS

Filed Sept. 20, 1930

2 Sheets-Sheet 2



INVENTOR  
Frederick P. Gardner  
BY Darby & Darby  
ATTORNEYS

## UNITED STATES PATENT OFFICE

1,959,757

## METHOD OF CLEANING FIBERS

Frederick P. Gardner, New York, N. Y., assignor  
to Fabricord, Inc., New York, N. Y., a corpora-  
tion of New York

Application September 20, 1930, Serial No. 483,213

7 Claims. (Cl. 19—24)

This invention relates to a method of cleaning or scutching fibers and has for its object the removal of the woody part and other substance from fiber bearing plants, such as flax, hemp, jute, ramie, and the like.

Under its broader aspect the invention includes the separation of the fibers from the non-fibrous woody or pithy and gummy matter by intense disruptive actions which are applied alternately on 10 the opposite sides of the fiber containing plants or straws. The disruptive action is applied in such a manner as to break up and whip out the undesired non-fibrous matter.

The disruptive action may be in the form of 15 whipping blows and is preferably applied in the direction of and along the length of the plant stalks or straws. The stalks or straws are held suspended, that is they are fed slowly in the direction of the whipping blows whereby the fiber it- 20 self is subjected to intense rippling or vibratory actions. The whipping action breaks up and the rippling or vibratory action shakes out the non-fibrous material from the fibrous material. The 25 intensity of the whipping action may be varied in different ways, as by increasing the amplitude of vibration of the fibrous material due to a difference of projections of the striking members which administer the whipping blows or the distance between the disrupting members. A fur- 30 ther way of varying the intensity of the action is by increasing, or decreasing, the rate at which the blows are administered to a definite portion of material fed. A further mode of varying the whipping actions is by varying the intervals at 35 which the blows are delivered, or by increasing or decreasing the oscillations of the rippling action on the plant stalks or straws as the same are moved forward. The intensity may be further varied by the manner in which the blows are de- 40 livered across the moving fiber bearing plants or stalks.

An important feature of applying the whipping blows is included in supplying proper cushioning means for the fibers over which the fibers travel, 45 when the whipping blows are applied thereto. The manner in which the fibers are cushioned has an important bearing on the effectiveness of the disruptive action administered by the whipping members. It also influences the rippling action 50 and I find that the cushioning members may be movable or stationary as the case may be. In either instance the disruptive action will be influenced by the cushioning members.

There are other ways which suggest themselves 55 to those versed in the art and I apply the disrupt-

tive actions to the fiber in the manner set forth by any suitable apparatus, such as is disclosed in the attached drawings, in which—

Figure 1 shows the fiber suspended in a vertical plane and subjected to whipping blows from alternate sides as the fiber is suspended and slowly permitted to travel past the whipping medium. The fiber in this instance is suspended in a vertical plane and is caused to travel over the cushioning members. The cushioning members 65 may be movable or stationary. It is obvious that instead of permitting the fiber to travel in a vertical plane it may be fed in a horizontal plane with the same effects.

In Figure 2 the fiber is fed either from a vertical 70 position or from a horizontal position over a movable cushioning bed, on the opposite side of which the whipping action is applied. The fiber is then deflected from its path and travels over a stationary cushioning bed while the whipping 75 action is applied to the opposite side of the fiber.

By referring to the drawings it will be noted that the fiber 10 is fed and suspended by a pair of rollers 11 so as to permit the fiber to travel forward at any desired speed suitable for the conditions at hand. A form of whipping member is illustrated by the beater roll 12, beater roll 12', etc. In Fig. 1 the beater rolls are applied alternately with the cushioning members on opposite sides of the moving fiber. The fiber itself is 85 passed over a movable cushioning member 13 which has supporting slats 14 of different sizes so as to cushion the fiber unevenly. This is for the purpose of applying a greater disruptive action to the fiber bearing plant. The beater roll 90 itself is supplied with beater blades 15 which also are of different sizes and are differently spaced so that the intensity of the beater action will be varied due to this irregularity of the beater blades. Obviously the rate at which the beater roll 12 95 rotates influences the effect of the beater action on the fibrous material. This arrangement will impart to the fiber bearing plant stalks intense vibratory action due to the high rate of speed at which the beater roll travels. This action obvi- 100 ously may be varied by the rate at which the roll is permitted to rotate or by the rate at which the fiber is fed over the cushioning bed.

In order to thoroughly effect cleaning to any desired degree the fiber is subjected to whipping 105 action from the opposite side, while the cushioning member is applied on the side which heretofore had been subjected to the whipping action. This alternate cushioning and whipping action may be varied to the desired degree in order to 110

meet the conditions under which the method is applied, that is to say, straws or fiber plants which are green, unretted and tough will require greater intensity of disruptive action than dry or retted fiber material. It should be noted, however, that my method will efficiently clean and soften fibers in the green (unretted) state or in the dry and ripe (retted) state.

The conditions under which the fiber is subjected to the disruptive actions as illustrated in the apparatus shown in Fig. 2 is substantially the same as that just described. The fiber however is deflected from its path and passed over a stationary cushioning member 16 whereby more intense scutching is obtained than in the movable cushioning member illustrated for example by the device shown at 17. In either of the constructions illustrated by Figs. 1 or 2 it is obvious that the intensity of the disruptive action may also be varied by increasing or decreasing the distance between the whipping members and the cushioning members. The method therefore is capable of great flexibility and is applicable to the cleaning or scutching of fibrous materials as described above.

In this connection the apparatus defined and disclosed above is merely being taken as illustrative, rather than as specific for the reason that other forms of apparatus might suggest themselves to those versed in the art.

What I claim, therefore, as new and useful is:

1. That method of cleaning fiber which comprises subjecting the fiber containing stalks or plants to a succession of rapid whipping blows of varying intensity first on one side of the fiber mass and then on the opposite side thereof.

2. That method of cleaning fiber which comprises subjecting the fiber containing stalks or plants to a succession of rapid whipping blows of varying intensity first on one side of the fiber mass and then turning the fiber mass and subjecting the same to a rapid succession of whipping blows of varying intensities on the other side thereof.

3. That method of varying the intensity of the scutching action on fiber bearing plants or straws which comprises feeding said plants at a varying rate and imparting thereto a succession of blows of varying intensity.

4. That method of cleaning fiber bearing plants or straws which consists in varying the degree of scutching by varying the amplitude of the vibrations imparted to the fiber bearing plants or straws.

5. That method of cleaning fiber bearing plants or straws which comprises varying the intensity of scutching by varying the force of the whipping blows on the moving fiber mass to impart intense rippling action thereto.

6. That method of scutching fiber bearing plants or straws which comprises varying the rate and intensity of scutching by varying the rate and number of whipping blows imparted to the moving fiber mass on alternately opposite sides.

7. That method of cleaning fiber bearing plants or straws by a rippling action which comprises varying the intensity of scutching by varying the rate at which the fiber mass is subjected to the rippling action.

FREDERICK P. GARDNER.